

## UNITED STATES PATENT OFFICE

2,606,131

FIREPROOF, WATERPROOF, FLEXIBLE  
SHEETING RESISTANT TO PENETRA-  
TION BY CHEMICAL WARFARE VESI-  
CANT AGENTSWilliam H. Aiken and Albert L. James, United  
States Army, assignors to the United States of  
America as represented by the Secretary of WarNo Drawing. Application August 19, 1943,  
Serial No. 499,246

5 Claims. (Cl. 117—137)

(Granted under the act of March 3, 1883, as  
amended April 30, 1928; 370 O. G. 757)

1

The invention described herein may be manufactured and used by or for the Government for governmental purposes, without the payment to us of any royalty thereon.

This invention relates, generally, to sheet material resistant to chemical warfare vesicant agents, and which is also fireproof and waterproof. The invention relates particularly to such sheet material formed by applying one or more layers of a coating composition comprising as its essential ingredients, a proteinaceous material and an ammonium alkyl or alkyloamino phosphate, together with certain other ingredients as will be described hereinafter.

The object of this invention, generally stated, is to provide sheet material in the form of coated papers and fabrics which is resistant to chemical warfare vesicant agents, capable of being produced on a quantity production basis from inexpensive readily available materials, flexible at low temperatures, not subject to blocking or becoming sticky at relatively high temperatures, and which is fireproof and waterproof to relatively high degrees. This material is particularly useful in war-time for the manufacture of such articles as military capes to protect individuals against vesicant spray from airplanes, and to serve as protective covering for materiel. The sheeting material of this invention also has many commercial uses such as for making emergency raincoats, waterproof curtains, greaseproof wrappings, fireproof curtains and decorations, fire-proof insulation, and the like.

More specific objects of this invention will be obvious, and certain others will be apparent from the following detailed description thereof.

Briefly stated, the invention consists in applying to a base sheet, such as a long-fibered paper of the kraft type, cellophane, or fabrics, one or more layers of a coating composition containing as its essential ingredients a proteinaceous material and an ammonium alkyl or alkyloamino phosphate, and certain other ingredients such as a plasticizing material, and a solvent. If desired, the coating may be finally overcoated with a thin plasticized layer of a water-resistant lacquer or sheet which will adhere thereto.

For a more complete understanding of the nature and scope of this invention, reference may be had to the following detailed description thereof setting forth by way of illustration certain specific formulas and embodiments.

The proteinaceous materials used in the coating compositions may be casein, glue, soybean

protein (alpha) and mazlein (zein), and the like. It has been found that certain ammonium alkyl and alkyloamino phosphates serve in the coating compositions not only as fireproofing agents but also as plasticizers, making possible the reduction or elimination of the amount of hygroscopic, polyhydroxy alcohols such as glycerine, sorbitol, and triethylene glycol, which serve as plasticizing agents.

By the term "phosphate" it is intended to include the salt of any one of the phosphoric or phosphorous acids, including ortho-phosphoric acid, meta-phosphoric acid, pyro-phosphoric acid, hypo-phosphoric acid, phosphorous acid, and hypo-phosphorous acid. The phosphate radicals of these different phosphoric and phosphorous acids are more or less equivalent for the purposes of this invention.

The three following examples give the formulas in parts by weight of coating compositions constituting specific embodiments of this invention in which casein constitutes the proteinaceous material:

## Example 1

100 parts casein  
10-20 parts ammonium hydroxide  
3-6 parts formalin  
100 parts monoethanolamine ethyl phosphate  
As desired, water

## Example 2

100 parts casein  
15 parts ammonium hydroxide  
6 parts formalin  
50-150 parts monoethanolamine ethyl phosphate  
700 parts water

## Example 3

100 parts casein  
15 parts ammonium hydroxide  
6 parts formalin  
50-125 parts monoethanolamine ethyl phosphate  
125-75 parts glycerine  
700 parts water

45 The above casein coating compositions may be prepared in any desired manner. That is, there is no particular significance in preparing the compositions according to any definite procedure. One satisfactory method of preparation, is to dissolve the ingredients in the water component with stirring and agitation. Preferably, the mixing is carried out at room temperature so as not to volatilize too much of the ammonium hydroxide.

In the above examples, monoethanolamine bu-

3

ethyl phosphate can be substituted for the monoethanolamine ethyl phosphate, with substantially the same results. However, this material does not appear to be quite as good a fireproofing agent as the monoethanolamine ethyl phosphate. Ammonium ethyl phosphate and ammonium butyl phosphate can also be satisfactorily substituted in the three above examples in place of the monoethanolamine ethyl phosphate. Likewise, monoethanolamine phosphate can be used as the phosphate ingredient in the three above examples. This latter material makes a satisfactory fireproof coating but does not make as good a plasticizer as the ethyl and butyl monoethanolamine phosphates.

The six following examples give the formulas in parts by weight of coating compositions forming additional specific embodiments of this invention wherein glue, soybean protein (alpha), mazlein-zein, and zein serve as the proteinaceous materials:

*Example 4*

100 parts glue (hide or bone)  
200-50 parts a phosphate selected from the group consisting of ammonium ethyl phosphate, ammonium butyl phosphate, monoethanolamine ethyl phosphate, monoethanolamine butyl phosphate, and monoethanolamine phosphate.  
100-1000 parts water

*Example 5*

100 parts glue (hide or bone)  
200-50 parts a hygroscopic, polyhydroxy alcohol selected from the group consisting of glycerine, 3 sorbitol, and the glycols  
50-200 parts a phosphate selected from the group consisting of ammonium ethyl phosphate, ammonium butyl phosphate, monoethanolamine ethyl phosphate, monoethanolamine butyl phosphate, and monoethanolamine phosphate 4  
100-1000 parts water

*Example 6*

100 parts soy protein (alpha)  
 15 parts ammonium hydroxide  
 50-200 parts a phosphate selected from the group  
 consisting of ammonium ethyl phosphate,  
 ammonium butyl phosphate, monoethanol-  
 amine ethyl phosphate, monoethanolamine butyl  
 phosphate, and monoethanolamine phosphate  
 500-1000 parts water

*Example 7*

100 parts soy protein (alpha)  
15 parts ammonium hydroxide  
200-50 parts a hygroscopic, polyhydroxy alcohol selected from the group consisting of glycerine, sorbitol, and the glycols  
50-200 parts a phosphate selected from the group consisting of ammonium ethyl phosphate, ammonium butyl phosphate, monoethanolamine ethyl phosphate, monoethanolamine butyl phosphate, and monoethanolamine phosphate  
500-1000 parts water

*Example 8*

100 parts mazein-zein  
 25-200 parts a phosphate selected from the group consisting of ammonium ethyl phosphate, ammonium butyl phosphate, monoethanolamine ethyl phosphate, monoethanolamine butyl phosphate, and monoethanolamine phosphate  
 300-1000 parts ethyl alcohol 65% to 92%

*Example 9*

100 parts zein  
200-25 parts glycols  
25-200 parts a phosphate selected from the group consisting of ammonium ethyl phosphate, ammonium butyl phosphate, monoethanolamine ethyl phosphate, monoethanolamine butyl phosphate, and monoethanolamine phosphate.

10 300-1000 parts ethyl alcohol 65% to 92%

The compositions of Examples 4 through 9 may be prepared in accordance with the manner outlined above for the compositions given in Examples 1, 2 and 3.

15 Examples 1, 2 and 3. In each of the nine specific coating compositions given above, the proteinaceous material may be wholly or partially replaced by other proteinaceous materials, such as any one of those given above. Likewise, the phosphate component in the nine above specific examples, may be partially or wholly replaced by other phosphates of the same class.

The phosphates of the class satisfactory for use in the coating compositions of this invention may be prepared by reacting in the proper proportions the desired phosphoric acid derivatives with ammonia or the desired amino derivatives. For example, monoethanolamine ethyl phosphate is prepared by reacting 118 parts of the ethyl phosphoric acid with 72.5 parts of monoethanolamine. These two materials are mixed slowly and heat is evolved making cooling necessary. The resulting mixture should be neutral to litmus when mixed with water. Monoethanolamine butyl phosphate is prepared in the same manner by reacting together 100 parts of butyl phosphoric acid and 54 parts of monoethanolamine. Likewise, ethyl phosphate is prepared by reacting together the proper proportions of ammonia and ethyl phosphoric acid, ammonium butyl phosphate is prepared by reacting ammonia and butyl phosphoric acid, and monoethanolamine phosphate is prepared by reacting together monoethanolamine and phosphoric acid.

45 In the above nine specific examples, water and ethyl alcohol were used as the solvent component of the coating compositions. It will be understood that in place of ethyl alcohol other low alcohols may be used such as methyl alcohol, 50 propyl alcohol and butyl alcohol.

The ammonium ethyl phosphates, ammonium butyl phosphates, and monoethanolamine ethyl and butyl phosphates, are all non-crystallizing, hygroscopic substances, which give fireproofness. Monoethanolamine phosphate is also non-crystallizing, but is not as hygroscopic as the other phosphates.

As stated, the presently preferred material on which the coating compositions of this invention are applied is a long-fibered paper exemplified by the grade generally known as kraft paper. This type of paper is comparable to tough wrapping paper and may have a weight of from 10 to 150 pounds per ream. However, cellophane also serves as a satisfactory base, as well as certain fabrics such as cotton cloth.

The coating compositions may be applied to the base sheet by conventional coating procedure. For example, the coatings may be applied on a large scale by means of the standard coating equipment now used in paper mills for the manufacture of coated paper. One or more layers of the coating compositions may be applied on one or both sides, with one layer being of one type

and another layer being of another type. Of course, the more layers applied to the sheet base, the greater will be the protection given to vesicant agents, and the greater will be the degree of fireproofness and waterproofness obtained.

The layers of the coating compositions of this invention may be overcoated with a thin plasticized layer of a water-resistant lacquering solution or sheet which will adhere thereto. Such an overcoating is particularly desirable where the sheeting material is to be exposed outdoors for extended periods. For example, the coated sheets may be overcoated with a thin layer of lacquer material such as ethyl cellulose, cellulose acetate, or nitrocellulose. One specific example of a sheet overcoating material is a nitrocellulose lacquer plasticized with dibutyl sebacate, or the various pelargonates plasticizers.

Desired pigment materials may be incorporated in the protein-phosphate coatings, or in the over-coating lacquers, or both.

When glue is used as the proteinaceous constituent in the coating compositions, it is preferably cured by admixture with, dipping in, or exposure to, formaldehyde fumes in accordance with known procedure for rendering glue resistant to water.

The sheet materials made according to the invention are characterized by being flexible at temperatures as low as 0° F., and by not blocking (sticking together when tiered) up to 150° F. The sheeting materials are resistant to liquid vesicants, such as mustard gas, nitrogen mustard, and lewisite, up to several hours.

By the expression "fireproof," it is intended to designate that degree of non-inflammability such that the sheeting materials of this invention will not sustain combustion by themselves after being ignited and the external flame is removed, and when the ambient atmosphere is at room temperature.

By the expression "waterproof," it is intended to designate that degree of water resistance ordinarily associated with such materials as shower curtains, raincoats, oilcloths, and the like.

Since certain further changes, modifications, and substitutions may be made in the foregoing embodiments, formulas, and methods of preparations, without departing from the scope of the invention, it is intended that all matter contained in the above description shall be interpreted as illustrative and not in a limiting sense.

We claim as our invention:

1. A fireproof, waterproof, flexible sheeting resistant to penetration by chemical warfare vesicant agents which comprises a water absorbent, gas absorbent cellulosic sheet having applied thereto as a coating at least one layer of a composition comprising an ammoniated water solution of formalin-cured casein, and a fireproofing and plasticizing agent of the class consisting of monoethanol phosphate, monoethanol ethyl

phosphate, monoethanol butyl phosphate, ammonium ethyl phosphate, and ammonium butyl phosphate, the casein and fireproofing and plasticizing agent being present in the ratio of 100 parts of the former to 50-150 parts of the latter, the casein having approximately from 3 to 6 parts of formalin incorporated with each 100 parts thereof and the solvent having therein approximately 10 to 20 parts of ammonium hydroxide per 700 parts thereof.

2. A fireproof, waterproof, flexible sheeting resistant to penetration by chemical warfare vesicant agents which comprises a water absorbent, gas absorbent cellulosic sheet having applied thereto as a coating at least one layer of a composition comprising an ammoniated water solution of formalin-cured casein, glycerine, and a fireproofing and plasticizing agent of the class consisting of monoethanol phosphate, monoethanol ethyl phosphate, monoethanol butyl phosphate, ammonium ethyl phosphate, and ammonium butyl phosphate, the casein, glycerine, and fireproofing and plasticizing agent being present in the ratio of 100 parts of the casein to 50-125 parts of the said agent, and 125 parts to 75 parts of glycerine respectively as to the said agent, the casein having approximately from 3 to 6 parts of formalin incorporated with each 100 parts thereof and the solvent having therein approximately 10 to 20 parts of ammonium hydroxide per 700 parts thereof.

3. A fireproof, waterproof, flexible sheet according to claim 1 wherein the fireproofing and plasticizing agent is monoethanolamine ethyl phosphate.

4. A fireproof, waterproof, flexible sheet according to claim 1 wherein the fireproofing and plasticizing agent is ammonium ethyl phosphate.

5. A fireproof, waterproof, flexible sheet according to claim 2 wherein the fireproofing and plasticizing agent is monoethanolamine ethyl phosphate.

WILLIAM H. AIKEN.  
ALBERT L. JAMES.

#### REFERENCES CITED

The following references are of record in the file of this patent:

#### UNITED STATES PATENTS

| Number    | Name      | Date          |
|-----------|-----------|---------------|
| 126,851   | Taylor    | May 14, 1872  |
| 1,966,271 | Twiss     | July 10, 1934 |
| 2,032,605 | Whitehead | Mar. 3, 1936  |
| 2,193,818 | Kajita    | Mar. 19, 1940 |
| 2,262,634 | Cobbs     | Nov. 11, 1941 |
| 2,338,664 | Nadeau    | Jan. 4, 1944  |

#### FOREIGN PATENTS

| Number | Country       | Date          |
|--------|---------------|---------------|
| 3,262  | Great Britain | Dec. 22, 1900 |